

## 1

2,993,745

METHOD OF AND COMPOSITIONS FOR  
BLEACHING IN ACID SOLUTIONSRowell R. Dorsett, Baltimore, Md., assignor of one-half  
to Mangels, Herold Company, Inc., Baltimore, Md., a  
corporationNo Drawing. Filed July 27, 1956, Ser. No. 600,400  
7 Claims. (Cl. 8—108)

This invention relates to the bleaching of nylon, cellulosic materials, regenerated cellulosic materials and fibers or filaments of the polyesters while at the same time inhibiting the degradation of such materials by the active or bleaching chlorine, and to bleaching compositions which are effective in acid solutions and contain an inhibiting agent to prevent degradation of the materials mentioned while being bleached.

This application is a continuation-in-part of my co-pending application Serial No. 517,069, filed June 21, 1955, now abandoned.

Materials such as nylon, cellulosic materials, regenerated cellulosic materials and fibers or filaments of the polyesters are very sensitive to bleaching agents and are degraded by them. Nylon in particular is very difficult to bleach and is degraded by alkaline bleaching compounds. There are compounds available which yield active or bleaching chlorine in both alkaline and acid solutions. But these compounds if not used in acid solution with agents inhibiting degradation by the active or bleaching chlorine, are very destructive of the type of materials above mentioned.

I have found that trichlorocyanuric acid and dichlorocyanuric acid when used in alkaline solutions will degrade materials such as nylon, cellulosic materials, regenerated cellulosic materials and fibers or filaments of the polyesters above mentioned. These bleaching agents, namely trichlorocyanuric acid and dichlorocyanuric acid will degrade these materials in alkaline solutions even when the inhibiting agents described infra are present in the bleaching solution. I have found that these bleaching agents will degrade the materials mentioned above in acid solution also unless the inhibiting agent to be described infra is present in the solution. To insure that the bleaching solutions will remain acidic in use, acidifying agents may be added to the solution in addition to the acidity supplied by the acid bleaching agents themselves.

It is therefore an object of this invention to provide a method of bleaching nylon, cellulosic materials, regenerated cellulosic materials and fibers or filaments of the polyesters in an acidic solution containing as the active bleaching agent trichlorocyanuric acid or dichlorocyanuric acid and an inhibiting agent selected from the molecularly dehydrated phosphates of the group consisting of the alkali metal phosphate glasses in which the ratio of  $M_2O$  to  $P_2O_5$  is from 0.5:1 to about 1.7:1, where M is sodium, potassium or ammonium and the crystalline alkali metal molecularly dehydrated phosphates such as the sodium or potassium tripolyphosphates ( $Na_5P_3O_{10}$  or  $K_5P_3O_{10}$ ), the sodium and potassium pyrophosphates ( $Na_2P_2O_7$  and  $K_2P_2O_7$ ) and the sodium and potassium acid pyrophosphates ( $Na_2H_2P_2O_7$  and  $K_2H_2P_2O_7$ ). In preparing the bleaching solution sufficient of the bleaching agent, either trichlorocyanuric acid or dichlorocyanuric acid, is added to provide in the solution the concentration of available chlorine desired for the particular bleaching job to be accomplished. For the ordinary domestic or household bleaching the concentration of available chlorine may be

## 2

of the order of one percent. For heavy duty bleaching such as encountered in commercial laundries the amount of the bleaching agent added may be such as will provide in the bleaching solution a concentration of from 500 p.p.m. to 250,000 p.p.m. of available chlorine. The concentration may be made lower than that or higher depending upon the amount of the bleaching agent—either trichlorocyanuric acid or dichlorocyanuric acid, required. To protect the materials bleached from degradation by the active or bleaching chlorine, an inhibiting agent selected from the group of the molecularly dehydrated phosphates above mentioned, may be added in amount sufficient to prevent degradation. The amount of molecularly dehydrated phosphate added may vary from about 1,000 p.p.m. to approximately 400,000 p.p.m. In any case the molecularly dehydrated phosphate added could vary from twenty-five pounds to sixty or seventy pounds per 100 pounds of water.

To the bleaching solution acidifying agents may be added in order to insure that the pH thereof will be below 7, preferably in the range from about 4.5 to 6.9.

Another object of the invention is to provide an effecting bleaching composition in which the effective or essential bleaching agent is selected from the class consisting of trichlorocyanuric acid and dichlorocyanuric acid and in which the inhibiting agent is a molecularly dehydrated phosphate selected from the group consisting of the alkali metal phosphate glasses above mentioned and the alkali metal tripolyphosphates and the alkali metal pyrophosphates, including the disodium dihydrogen pyrophosphate and the dipotassium dihydrogen pyrophosphate.

A further object of the invention is to provide a bleaching composition containing as its effective bleaching agent a compound selected from the group consisting of trichlorocyanuric acid and dichlorocyanuric acid and a molecularly dehydrated phosphate for inhibiting degradation; to provide a composition which is stable under ordinary conditions of storage and transportation and which when dissolved in water will yield solutions suitable for bleaching, sterilizing and disinfecting and particularly for the bleaching of materials such as nylon, cellulosic materials, regenerated cellulosic materials and fibers or filaments of the polyesters.

Other objects of the invention are to provide a composition as above set forth which is useful as a disinfecting detergent for laundry and other purposes, as a bleaching detergent composition for laundry and other purposes where protection against degradation of the bleached fabrics is essential.

The above and other objects of the invention will be apparent to those of ordinary skill in the art to which the invention pertains from the following description.

A bleaching composition embodying the invention may be prepared by mixing a compound of the group consisting of trichlorocyanuric acid and dichlorocyanuric acid and an agent that is effective to inhibit degradation of the materials such as nylon, cellulosic materials, regenerated cellulosic materials and fibers or filaments of the polyesters. The trichlorocyanuric acid and the dichlorocyanuric acid are available having a high available active chlorine content. If these materials have 85 percent available chlorine, approximately 1.12 pounds thereof in 100 pounds of water will yield about 1 percent available chlorine. For the ordinary composition that would be used in the household, it would contain sufficient of the active acidic bleaching agent to provide about 1 percent available chlorine, and sufficient inhibiting agent to

prevent degradation of the fabrics bleached in the solution. For the ordinary domestic or household use the composition may contain materials other than the bleaching and inhibiting agent to provide such bulk that when a cup full of the composition is added to the tub of the average washing machine, the available chlorine in the solution will be about 1 percent.

For heavier duty bleach operations, the content of the active bleaching agent may be increased as much as practical requirements, dictate, as when 5 percent to 15 percent or more of available chlorine is desired. In any case, whether the quantities of the composition used produce relatively low or relatively high concentrations of available or active chlorine, the amount of agent in the composition which prevents degradation of the above mentioned materials will be such as to effectively achieve that result, namely the prevention of degradation.

The compositions in general may consist of the active bleaching agent—either the trichlorocyanuric acid or the dichlorocyanuric acid, a molecularly dehydrated phosphate, an acidifying agent and a filler or neutral material to give it bulk so that the composition may be used with economy and in the concentrations desired without accurate measurement.

The acidifying agents may be selected from among the compounds such as sodium bisulphate, acetic acid, diacetic acid, sodium diacetate, citric acid, sulfamic acid and oxalic acid. The acidifying agents may also include monoalkali metal dihydrogen phosphate such as the sodium and potassium dihydrogen phosphate.

The composition as above stated will contain a molecularly dehydrated phosphate selected from the group of phosphates above described. For storage purposes, that is stability in storage, the crystalline alkali metal molecularly dehydrated phosphates are preferred to the molecularly dehydrated glassy phosphates.

The active bleaching agent i.e. either trichlorocyanuric acid or dichlorocyanuric acid, may be used to form a bleaching detergent composition also. In such a composition, the detergent shall be one that is operative in acid solution, and which does not when in the composition, deteriorate in storage, cause the acidic bleaching agent to break down or which will not itself decompose in the presence of the active bleaching agent. I have found that Petro AA which is an alkyl naphthalene sulfonate, in powder form 98 percent active, to be well suited for the formulation of the bleaching detergent composition as it provides a product that is stable in storage, has a long shelf life, remains free-flowing and does not deleteriously affect the active bleaching agent.

The following are examples of the bleaching composition:

#### Example I

22.5 parts by weight of trichlorocyanuric acid 85 percent active  
50 parts by weight sodium tripolyphosphate ( $Na_5P_3O_{10}$ )  
27.5 parts by weight sodium sulfate

The pH of a one percent tap water solution of the above composition (Example I) is 6.5 where the tap water itself had a pH of about 8.2. The composition of Example I will provide an available chlorine content in a bleaching solution of 19.125 or approximately 20 percent where 100 parts by weight of the composition is used in 100 parts by weight of water.

The composition of Example I is suitable for commercial bleaching applications such as are encountered in commercial laundries.

#### Example II

22.5 parts by weight trichlorocyanuric acid 85 percent active chlorine  
30 parts by weight sodium tripolyphosphate  
30 parts by weight monosodium dihydrogen phosphate  
17.5 parts by weight sodium phosphate glass

A one percent solution of the composition of Example II in tap water will have a pH of about 5.8 and will provide an available chlorine content in a bleaching solution of about 20 percent. This composition is useful in industrial sanitizing applications and for heavy duty bleaching.

#### Example III

11 parts by weight trichlorocyanuric acid 85 percent available chlorine  
10 parts by weight sodium tripolyphosphate  
15 parts by weight monosodium dihydrogen phosphate  
54 parts by weight sodium sulfate

The pH of a one percent solution in tap water of the above Example III is about 6.1, the tap water having a pH of about 8.2. The composition will provide an available chlorine content in the bleaching solution of about 10 percent. In computing the available chlorine content in the solution it is to be remembered that 1 pound of the trichlorocyanuric acid 85 percent available active bleaching chlorine will provide .85 percent of available chlorine in the solution.

The above composition is useful in heavy duty bleaching and in industrial sanitizing applications.

25

Example IV

8.0 parts by weight trichlorocyanuric acid 85 percent available active or bleaching chlorine  
35.0 parts by weight sodium tripolyphosphate  
30 42.0 parts by weight of monosodium dihydrogen phosphate  
15 parts by weight Petro AA

As stated supra Petro AA is an alkyl naphthalene sulfonate 98 percent active and is a powder.

35 The pH of a 1 percent solution in tap water of Example IV is about 6.2 and it will provide an available chlorine content in aqueous solution of about 7 percent when sufficient of the composition is added to the solution to provide approximately 8 parts by weight of the trichlorocyanuric acid for each 100 parts by weight of water.

In the foregoing examples dichloro-cyanuric acid may be substituted for the trichlorocyanuric acid in substantially the same proportions by weight. The dichloro-cyanuric acid has about 65% to 70% available chlorine according to the technical literature of manufacturers of that product.

Furthermore, in the foregoing examples an acidifying agent selected from the group consisting of sodium bisulfate, acetic acid, diacetic acid, sodium diacetate, citric acid, sulfamic acid and oxalic acid may be added to the compositions to insure that the solutions of the compositions will be acidic in use and provide a pH in the bleaching solutions ranging from pH about 4.5 to about 55 6.9. It is preferred that the pH range be maintained between 5.5 and 6.1.

Sodium bicarbonate may be effectively used with the acidifying agent.

From the foregoing examples it will be apparent that the proportions of the trichlorocyanuric acid and the dichloro-cyanuric acid used in the compositions may vary from about 8 parts by weight to about 22.5 parts by weight. The upper concentration in parts by weight of the trichlorocyanuric acid or the dichloro-cyanuric acid may be higher than 22.5 where extremely heavy duty bleaching solutions are required.

Trichlorocyanuric acid is sometimes referred to in the literature as trichloroisocyanuric acid, but so far as is known the trichloroisocyanuric acid is identical with the trichlorocyanuric acid.

The compositions of Examples I, II and III are useful in the preparation of bleaching solutions. The composition of Example IV is one that is both a detergent and a bleaching composition.

The bleaching compositions as above stated are inhibited against the degradation of materials such as nylon, cellulosic materials, regenerated cellulosic materials and others herein identified. The following data are test results on cotton sheeting unbleached but wet out and used in the test. In the test the strength of the warp and the filling was measured before bleaching. The following tabulations indicate how the tests were performed and the results:

| Unbleached                                                                                                                                                                                                  | Warp | Filling |
|-------------------------------------------------------------------------------------------------------------------------------------------------------------------------------------------------------------|------|---------|
| Strength in pounds on Scott Tester.....                                                                                                                                                                     | 80   | 60      |
| Solution containing 500 parts per million of trichlorocyanuric acid solution adjusted to pH of about 5.5—goods bleached 30 minutes at 160° F.....                                                           | 54   | 32      |
| Solution containing 500 parts per million of trichlorocyanuric acid and a 20% solution of monosodium dihydrogen phosphate the solution adjusted to pH of about 5.5—goods bleached 30 minutes at 160° F..... | 78   | 59      |
| Bleaching solution of calcium oxychlorite (CaOCl) 500 parts per million in solution pH 9.6—goods bleached 30 minutes at 160° F.....                                                                         | 27   | 19      |

The tests of the above tests show the initial strength of the unbleached goods, the loss in strength of the warp and the filling where the trichlorocyanuric acid did not contain a phosphate, the strength after bleaching with phosphate in solution, the value showing only an insignificant loss in strength on the warp and the filling.

The loss in strength resulting from the use of calcium oxychloride was very significant and substantial.

The following shows the results of bleaching use-yellowed nylon garments in solution containing the trichlorocyanuric acid and sodium "Lorol" sulfate. The bleach bath contained 0.1% sodium "Lorol" sulfate and 1.13% trichlorocyanuric acid. The bleach bath was at a temperature of 70° C., and the bleach cycle was two hours.

A set of seven (7) use-discolored fabrics having an average yellowness of 7.1 +b units as measured on a differential colorimeter had an average yellowness of 3.1 +b units after bleaching in the above solution. This is an acceptable shade of whiteness.

In another test the following use-yellowed nylon garments having the +b value of whiteness indicated were bleached in a solution containing about 1.13% by weight of the trichlorocyanuric acid.

| Garment | +b Value | After bleaching +b Value |
|---------|----------|--------------------------|
| blouse  | 2.5      | 2.5                      |
| shirt   | 3.3      | 2.6                      |
| slip    | 3.7      | 2.4                      |
| shirt   | 4.2      | 3.1                      |
| Do      | 4.3      | 2.8                      |
| slip    | 4.9      | 3.1                      |
| Do      | 5.3      | 3.6                      |
| shirt   | 5.3      | 3.0                      |
| blouse  | 6.1      | 2.8                      |
| shirt   | 6.9      | 3.1                      |
| slip    | 8.0      | 3.8                      |
| sweater | 11.7     | 4.0                      |

After bleaching, the blouse having the +b value of 2.5 had a reflectance b value of 2.5. The average +b values for the other garments was approximately 3.06. The +b values for the respective garments after bleaching are indicated in the column headed "After bleaching +b value."

Seven use-yellowed nylon garments were bleached in a solution containing the trichlorocyanuric acid in amount to give about 1% available chlorine and containing a molecularly dehydrated phosphate within the amounts indicated in the Examples I to IV, and adjuvants as indicated in the following table. The table gives the pH of the solutions and the average b values (the degree of whiteness resulting after bleaching). Trichlorocyanuric

acid was present in each of the following in amount sufficient to yield about 1% available chlorine.

| Garment | Adjuvants                                                                                                                                | pH of Solution | Avg. b Value |
|---------|------------------------------------------------------------------------------------------------------------------------------------------|----------------|--------------|
| 1.....  | Na <sub>2</sub> SO <sub>4</sub> , Na <sub>2</sub> H <sub>2</sub> P <sub>2</sub> O <sub>7</sub> , NaNO <sub>3</sub> , sulfamic acid       | 3.2            | 2.8          |
| 2.....  | Na <sub>2</sub> SO <sub>4</sub> , Na <sub>2</sub> H <sub>2</sub> P <sub>2</sub> O <sub>7</sub> , NaNO <sub>3</sub> , less sulfamic acid. | 5.0            | 3.4          |
| 3.....  | Na <sub>2</sub> SO <sub>4</sub> , Na <sub>2</sub> H <sub>2</sub> P <sub>2</sub> O <sub>7</sub> , Na diacetate.....                       | 5.3            | 3.6          |
| 4.....  | Na <sub>2</sub> SO <sub>4</sub> , "Calgon" benzoic acid.....                                                                             | 3.9            | 3.3          |
| 5.....  | Na <sub>2</sub> H <sub>2</sub> P <sub>2</sub> O <sub>7</sub> , synthetic detergent.....                                                  | 5.8            | 3.1          |
| 6.....  | Acetic acid.....                                                                                                                         | 5.5            | 3.3          |
| 7.....  | Na "Lorol" sulfate (0.2%), Acetic acid.....                                                                                              | 3.5            | 2.1          |

Similar tests have indicated that similar results are obtainable by the employment of dichlorocyanuric acid in lieu of trichlorocyanuric acid.

From the foregoing it is apparent that a process has been provided whereby material such as nylon, cellulosic materials, regenerated cellulosic materials and fibers or filaments of the polyesters may be bleached or washed and bleached effectively and safely in acidic solutions containing trichlorocyanuric acid or dichlorocyanuric acid without suffering any substantial loss of strength through degradation.

It is also apparent that effective bleaching compositions which are inhibited against the degradation of the above mentioned materials, including bleaching and detergent compositions having the same properties has been provided.

Having thus described the invention it will be apparent to those of ordinary skill in the art to which the invention pertains that various modifications and changes may be made in the described method and the examples of the compositions without departing from either the spirit or the scope of the invention.

Therefore, what is claimed as new and desired to be secured by Letters Patent is:

1. The method of bleaching fibers and filaments of nylon, cellulose, regenerated cellulose, and polyesters which consists of preparing an aqueous solution of an active bleaching agent of the group consisting of trichlorocyanuric acid and dichlorocyanuric acid in amount sufficient to provide about 1% to about 25% of available chlorine, and a degradation inhibiting agent selected from the class of phosphate consisting of alkali metal molecularly dehydrated phosphate glass, alkali metal tri-polyphosphate and alkali metal pyrophosphate, including alkali metal acid pyrophosphate, adjusting the pH of the solution to a value from about pH 4 to 6.9, soaking the materials to be bleached in the solution, rinsing, and removing the materials from the bleach and drying the same.

2. The method of claim 1 in which the pH of the solution is maintained between pH 5 and pH 6.2 by monoalkali metal dihydrogen phosphate.

3. A bleaching composition for bleaching in acid solution fibers and filaments of nylon, cellulose, regenerated cellulose and polyesters which comprises:

(a) An 8 to 25% by weight acid bleaching compound of the class consisting of trichlorocyanuric acid and dichlorocyanuric acid computed on an 85% available chlorine basis,

(b) Alkali metal molecularly dehydrated phosphate 25 to 50 percent by weight, and

(c) The balance consisting of a compound selected from the group consisting of sodium sulfate, and monoalkali metal dihydrogen phosphate.

4. A bleaching composition comprising:

(a) Trichlorocyanuric acid (85% available chlorine) 8 to 22.5 percent by weight,

(b) Alkali metal molecularly dehydrated phosphate 25 to 50 percent by weight, and

(c) An acidifying agent in amount sufficient to maintain a 1% solution of the composition at a pH value from 4.5 to about 6.5.

5. A bleaching and detergent composition comprising 8 to 25% by weight of a bleaching agent of the group consisting of trichlorocyanuric acid and dichlorocyanuric acid computed on an 85% available chlorine basis, and molecularly dehydrated phosphate 25 to 50 percent by weight and a detergent consisting about 15% by weight of alkyl naphthalene sulfonate 98% active, the balance consisting of acidifying agents.

6. A bleaching composition for nylon, cellulosic and similar materials having as its active bleaching agent a compound of the class consisting of trichlorocyanuric and dichlorocyanuric acids and a degradation inhibiting agent selected from the class of alkali metal molecularly dehydrated phosphate glasses, the crystalline tri-polyphosphates and the crystalline pyrophosphates, the ratio of the bleaching agent computed on an 85% available chlorine basis to inhibiting agent in percent by weight being in the range of 8:20 to 25:50; and having a pH in 10% solution between 5 and 6.

10

15

7. A composition as in claim 6 containing an acidifying agent in amount sufficient to maintain the pH of a 1% solution of the composition between 4.5 and 6.5.

## References Cited in the file of this patent

## UNITED STATES PATENTS

|           |                |                |
|-----------|----------------|----------------|
| 1,892,548 | Feibelmann     | Dec. 27, 1932  |
| 2,075,913 | Sanchez        | Apr. 6, 1937   |
| 2,121,501 | Hershman       | June 21, 1938  |
| 2,166,362 | MacMahon       | July 18, 1939  |
| 2,171,901 | Wilson et al.  | Sept. 5, 1939  |
| 2,422,255 | Peters         | June 17, 1947  |
| 2,578,270 | Strain         | Dec. 11, 1951  |
| 2,607,738 | Hardy          | Aug. 19, 1952  |
| 2,611,700 | Brunner et al. | Sept. 23, 1952 |

## FOREIGN PATENTS

|         |       |               |
|---------|-------|---------------|
| 406,431 | Italy | Nov. 23, 1943 |
|---------|-------|---------------|